

## UNITED STATES PATENT OFFICE

2,425,501

## PREVENTION OF CRAZING OF FLASH HEATED SHAPES OF POLYSTYRENE

Fred E. Wiley, Hartford, Conn., assignor to Plax Corporation, Hartford, Conn., a corporation of Delaware

No Drawing. Application May 4, 1943,  
Serial No. 485,650

8 Claims. (Cl. 18—47.5)

1

This invention relates to the production of articles of polystyrene by processes which involve "flash heating" which term as used herein means an operation in which the surface of the polystyrene is rapidly heated to or above, usually substantially above, the transition temperature of the material which is about 180° F. Flash heating may occur in buffing, polishing or machining operations or in die drawing shapes of polystyrene in a highly heated die which may be heated to 580–600° F. Die drawing may be used to obtain articles of accurate shapes and dimensions and having a high polish.

Flash heating of shapes of polystyrene causes crazing or cracking upon cooling of the shapes.

I have discovered that crazing or cracking resulting from flash heating of polystyrene shapes may be prevented by a certain heat treatment. This treatment involves heating a shape in a temperature range above the transition temperature, preferably 194–221° F., for a certain period of time before flash heating, then immediately flash heating the shape, then immediately quenching the shape in a cold bath, preferably a bath at a temperature below room temperature, for example, 40–50° F., and holding the shape in the quenching bath for a certain minimum time. The initial heating of the shape is effected in a certain minimum time to soften the sub-surface material but for an insufficient time to soften the core of the shape to such an extent that the shape can be permanently deformed, or in the case of a rod, permanently stretched until it has become undersized as might occur in die drawing.

This treatment prevents surface crazing and cracking of the shape during and after flash heating as well as preventing deformation or stretching of the shape which might occur if the heating should be conducted at a higher temperature and/or longer time.

Subsequent to the above steps the shape may be further treated to mechanically stabilize it, as by heating the shape to or above the transition temperature, and then cooling it at a rate predetermined to produce in the shape a selected maximum stress which will permit machining the shape or will permit it to be used without cracking or failure, as a result of internal mechanical stress.

## Example

A rod of polystyrene is heated to a temperature of approximately 194–221° F., preferably in a bath of ethylene glycol, for a period of time not less than about one-quarter of the time necessary to obtain uniformity of temperature

5 throughout the shape within 1° F. The length of the heating period is less than the time required to heat the core of the rod to such an extent that when the rod is subjected to flash heating in a drawing die and is drawn therethrough it would stretch permanently and become undersized. After heating the rod within the limits of time above stated, the shape is immediately flash heated as by die drawing it through a die heated 10 to 580–600° F. Immediately after the flash heating, the rod is quenched in a cold water bath which may be maintained at a temperature of 40–50° F. The rod is held in the quenching bath for a minimum period of time, preferably not less than one-half the approximate time necessary to obtain uniform temperature throughout the rod 15 within 1° F. Following this treatment, the rod may be removed from the bath. The rod or other shape should not be allowed to remain out of the 20 heating medium and the quenching bath any longer than necessary before and after flash heating and usually this period of time is not over 1½ minutes.

It will be understood that changes may be 25 made in the above described procedure and my novel process may be used in treating various materials containing polystyrene or the like, without departing from the scope of the appended claims.

30 Having thus described my invention, what I claim is:

1. The process of preventing crazing of a flash heated shape of polystyrene which comprises first heating the shape at a temperature of approximately 194–221° F., flash heating the shape at a temperature substantially above said first named temperature, and quenching the shape.

2. The process of preventing the crazing of a flash heated shape of polystyrene which comprises heating the shape to a temperature of approximately 194–221° F. for a period of time not less than approximately one-fourth of the time required to obtain uniformity of temperature throughout the shape within 1° F., flash heating 40 the shape at a temperature substantially above said first-named temperature, and immediately quenching the shape.

3. The process of preventing the crazing of a flash heated shape of polystyrene which comprises initially heating the shape at a temperature of approximately 194–221° F., flash heating the shape at a temperature substantially above said first-named temperature, and quenching the shape in a bath maintained at a temperature of approximately 40–50° F.

34

4. The process of preventing the crazing of a flash heated shape of polystyrene which comprises initially heating said shape at a temperature of approximately 194-221° F. for not less than about one-fourth of the time necessary to obtain uniformity of temperature throughout the shape within 1° F. and for an insufficient period of time to heat the core of the shape enough to permit permanent deformation of stretching of the shape, flash heating the shape at a temperature substantially above said first named temperature, and immediately quenching the shape.

5. The process of preventing the crazing of a flash heated shape of polystyrene which comprises heating said shape in a liquid bath at a temperature of approximately 194-221° F. for not less than about one-quarter of the time necessary to obtain uniformity of temperature in the shape within 1° F. and for a period of time less than that in which the core of the shape would be heated sufficiently to permit permanent deformation or stretching, immediately flash heating the shape at a temperature substantially above said first-named temperature, and immediately thereafter quenching the shape in a bath having a temperature not higher than approximately 50° F.

6. The process of preventing the crazing of a flash heated shape of polystyrene which comprises initially heating said shape at a temperature of approximately 194-221° F. for not less than about one-fourth of the time necessary to obtain uniformity of temperature within 1° F. for an insufficient time for the core of the shape to be heated enough to permit permanent deformation or stretching of the shape, immediately flash heating the shape at a temperature substantially above said first-named temperature, immediately quenching the shape in a bath

4

maintained at a temperature not higher than approximately 50° F. and holding the shape in the quenching bath for not less than approximately one-half the time necessary to obtain uniform temperature throughout the shape within 1° F.

7. The process of preventing the crazing of a flash heated shape of polystyrene which comprises first heating the shape to a temperature of approximately 194-221° F., immediately flash heating the shape at a temperature of approximately 580-600° F., and immediately quenching the shape.

8. The process of preventing crazing of a flash heated shape of polystyrene which comprises first heating the shape at a temperature of approximately 194-221° F., immediately flash heating the shape by drawing it through a die heated to a temperature of approximately 580-600° F., and thereafter immediately quenching the shape.

FRED E. WILEY.

#### REFERENCES CITED

The following references are of record in the  
5 file of this patent:

UNITED STATES PATENTS

| Number    | Name           | Date          |
|-----------|----------------|---------------|
| 2,194,313 | Loomis         | Mar. 19, 1940 |
| 2,239,780 | Fidentscher    | Apr. 29, 1941 |
| 2,166,215 | Lloyd          | July 18, 1939 |
| 2,205,449 | Wiley          | June 25, 1940 |
| 1,683,402 | Ostromislensky | Sept. 4, 1928 |
| 2,145,119 | Littleton      | Jan. 24, 1939 |
| 2,177,633 | Blackard       | Oct. 31, 1939 |
| 2,311,818 | Dawson         | Feb. 13, 1943 |

#### OTHER REFERENCES

Ind. & Eng. Chem., Sept. 1942, pages 1052 to  
056